

## UNITED STATES PATENT OFFICE

2,243,765

## TREATMENT OF CELLULOSIC TEXTILE MATERIALS

Thomas Henry Morton, Braintree, England, assignor to Courtaulds Limited, London, England, a British company

No Drawing. Application April 18, 1940, Serial No. 330,425. In Great Britain April 4, 1939

3 Claims. (Cl. 260—212)

This invention relates to the treatment of cellulose textile materials with formaldehyde.

It is well known to treat cellulose materials with formaldehyde with the object of obtaining various effects. For example, Eschalier in British Specification No. 25,647/06 has disclosed a process for strengthening cellulose threads, films and the like which consists in impregnating the materials with a solution containing an aldehyde which may be formaldehyde and an acid or acid-reacting substance, and then treating under dehydrating conditions.

It has now been found that a different type of product can be obtained from cellulose and formaldehyde by treating cellulose with an aqueous solution of formaldehyde containing a small proportion of an acid catalyst under such conditions of time and temperature that the reaction is allowed to approach its equilibrium. In order to isolate the compound of cellulose and formaldehyde produced according to this invention, it is necessary to remove the uncombined formaldehyde and the acid catalyst before drying it, or subjecting it to any other dehydrating conditions.

In carrying out the process of this invention the proportion of the solution of formaldehyde to the cellulose must be at least such that the cellulose is always in a fully swollen state. Generally it is preferred to have present however a considerably greater quantity of water than is necessary merely to produce this swollen state.

The time and temperature of the treatment with the solution of formaldehyde and acid catalyst will vary with one another, the time required increasing rapidly as the temperature diminishes. The rate of absorption of formaldehyde by the cellulose will also depend upon the concentration of the acid and of the formaldehyde in the treating solution.

Using a solution containing 40 per cent of formaldehyde and sulphuric acid sufficient to give a 'normal' solution the reaction is substantially complete in 10 minutes at 80° centigrade, in 1 hour at 60° centigrade and in 24 hours at 24° centigrade. Using a deconormal solution of sulphuric acid containing 40 per cent of formaldehyde a time of 1 hour is required at 80° centigrade to reach the same stage.

When it is desired to isolate the product by washing and drying, the washing must be thorough and is preferably carried out first in cold and then in hot running water, while the drying is preferably effected at a temperature round about 100° centigrade.

The cellulose material may be in the form of cotton linters, bleached wood pulp, or yarn or fabric prepared from natural or artificial fibres.

The product obtained is different in many of its properties from that obtained by heating cellulose with formaldehyde and then dehydrating. For example, whereas it has been stated that when using Eschalier's process about 0.2 to 0.3 per cent of formaldehyde is combined with the cellulose, the product obtained according to the present invention may contain up to 3 to 4 per cent, or even more, of combined formaldehyde, although we do not limit our invention to the production of compounds containing this proportion of formaldehyde. If, for example, the treating solution contains a smaller proportion of formaldehyde, the equilibrium is reached when smaller proportions of formaldehyde are combined with the cellulose. For instance, if the treating solution contains about 20 per cent of formaldehyde, the reaction equilibrium will be reached when the cellulose contains about 1 per cent of methylene oxide. The great differences between the products obtained according to the present invention, and that described by Eschalier in the aforesaid British Specification No. 25,647/06, and which is generally termed "sthenosaged" cellulose, are that the products obtained according to the present invention show no increase in wet strength and possess a high water imbibition, no increased resistance to creasing and a slightly increased affinity towards some direct dyes, all of which effects are contrary to those possessed by sthenosaged cellulose products.

The product obtained according to the present invention reacts with nitrogenous compounds such as cyanamide and salts of tertiary bases, for example pyridine and triethanolamine, to give materials having a good affinity for those dyes normally used for dyeing wool. Its use in this connection is described in the co-filed joint application of John Boulton and myself, Serial No. 330,424.

By heating the formaldehyde-cellulose product of the invention in the presence of an acid catalyst under dehydrating conditions, the previously known sthenosaged product with different properties can be obtained.

The following example illustrates one method of carrying out the present invention although the invention is not restricted to this example.

## Example

55 A fabric woven from yarn prepared from the

staple fibre marketed under the registered trade-mark "Fibro" is immersed in 30 times its volume of a 40 per cent solution of formaldehyde acidified with sufficient sulphuric acid to form a "normal" solution, at 80° centigrade for 10 minutes. The fabric is then removed from the solution and washed, first in cold and then in hot running water until all traces of uncombined formaldehyde and sulphuric acid are removed. It is then dried at 105° centigrade for 10 30 minutes.

What I claim is:

1. The production of compounds of cellulose with formaldehyde by treating cellulose with an aqueous solution of formaldehyde containing a 15 small proportion of an acid catalyst under such conditions of time and temperature that the reaction is allowed to approach its equilibrium, the proportion of the solution of formaldehyde to the cellulose being such that the cellulose is 20 always in a fully swollen state, said solution containing 40% formaldehyde, said catalyst being sulphuric acid in decinormal to normal solution, said time being from 10 minutes to 24 hours, and said temperature being from 24° C. to 80° C. 25

2. The production of compounds of cellulose with formaldehyde by treating cellulose with an aqueous solution of formaldehyde containing a small proportion of an acid catalyst under such conditions of time and temperature that the reaction is allowed to approach its equilib- 30

rium, the proportion of the solution of formaldehyde to the cellulose being such that the cellulose is always in a fully swollen state, said solution containing 40% formaldehyde, said catalyst being sulphuric acid in decinormal to normal solution, said time being from 10 minutes to 24 hours, and said temperature being from 24° C. to 80° C., removing the uncombined formaldehyde and the acid catalyst from said compound, and thereafter subjecting said compound to dehydration.

3. The production of compounds of cellulose with formaldehyde by treating cellulose with an aqueous solution of formaldehyde containing a small proportion of an acid catalyst under such conditions of time and temperature that the reaction is allowed to approach its equilibrium, the proportion of the solution of formaldehyde to the cellulose being such that there is present a considerably greater quantity of water than is necessary merely to produce a fully swollen cellulose, and the cellulose is thereby always in a fully swollen state, removing the uncombined formaldehyde and the acid catalyst from said compound, and thereafter subjecting the compound to dehydration, said solution containing 40% formaldehyde, said catalyst being sulphuric acid in decinormal to normal solution, said time being from 10 minutes to 24 hours, and said temperature being from 24° C. to 80° C.

T. H. MORTON.